

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## REFINED WOOD PULP OF LOW PENTOSAN CONTENT

No Drawing.

Application filed March 14, 1930. Serial No. 435,962.

This invention relates to the production of a refined wood pulp, and more especially one which is of exceedingly low pentosan content, of high alpha cellulose content, and of 5 low solution viscosity, if desired. Such a product, in addition to being an excellent papermaking material, is eminently suitable for use as a raw material for nitration, acetylation, or the like, in cases where it is desirable 10 that the cellulose derivatives be soluble to form solutions of high clarity but of low viscosity. Especially in the case of the acetates, it has been found that the presence of pentosans much above 1% in the fiber used 15 as a raw material for acetylation is largely responsible for opacity or cloudiness in solutions prepared from the acetylated product, as the use of cellulose fibers of high alpha cellulose content and containing less than 20 1% of pentosans in the preparation of cellulose acetates makes possible the production of cellulose acetate solutions of clarity and sparkle.

In producing refined pulps from wood or 25 kindred raw cellulosic materials, it has generally been the practice to prepare a raw wood pulp such as sulphite or kraft, and then to dissolve non-alpha cellulose components from such pulp by the use of alkaline 30 liquors. Such a process does not result in a product of minimum pentosan content, as the usual cooking liquors employed for liberating the fiber from wood are incompletely reactive upon the pentosans, and the resulting 35 raw pulp, which contains a substantial residue of pentosans is only partially freed from this impurity by alkaline liquors which, too, are only partly effective in their reaction thereupon.

40 I have found that if wood or kindred raw cellulosic material is treated or cooked in a liquor containing substantially only acid such as sulphurous and/or sulphuric, and is then cooked in an alkaline liquor containing 45 comparatively strong alkalies such as caustic soda and/or sodium sulphide, it is possible to produce a final product of an alpha cellulose content of about 96% or greater and of a pentosan content of less than 1%. 50 Such a product may be produced in a form

which is readily bleachable to high whiteness with a low bleach consumption. In bleached or unbleached condition, it may, if desired, be characterized by an exceedingly low solution viscosity, for instance, one which 55 ranges from 0.2 to 1.0, as against a value of from 40 to 200 in the case of raw sulphite or kraft pulp. This low solution viscosity renders the product suitable for conversion into cellulose derivatives without necessitating 60 one or more special treatments such as have heretofore been employed in lowering the solution viscosity of the cellulose fiber or the derivative prepared therefrom. Apparently 65 the use of substantially only acid in the initial treatment results in an effective hydrolysis of the pentosans into soluble sugars or other reaction products which are readily soluble in alkaline cooking liquors, but the initial treatment or cook need not be carried 70 out to complete fiber liberation, even when this is possible, as when sulphurous acid solutions are used, in order to avoid chemical injury to the wood fibers such as takes place 75 when they undergo a high temperature treatment in the form of pulp in a strongly acid liquor. Evidently the initial acid treatment transforms the alpha cellulose to a form profoundly different from that present in wood 80 pulp such as kraft or sulphite or raw cotton, for not only is the final product of surprisingly low solution viscosity when tested by the usual cuprammonium cellulose solution standard, but other derivatives, such as the nitrocelluloses prepared therefrom, 85 have even lower solution viscosity than similar derivatives prepared from other fibers whose cuprammonium cellulose solution viscosity has been lowered by one or more special treatments to the same value as that 90 possessed by a cuprammonium cellulose solution prepared therefrom.

In carrying out the initial treatment of the wood with a liquor containing substantially only acid, various acids and/or acid 95 salts, and various conditions of treatment may be used. The acids or acid salts employed, however, are comparatively strong or highly ionized in aqueous solution, and to this end mineral acids such as sulphuric, sul-

phurous, nitric, and hydrochloric, or acid salts of these acids, are suitable, as they effect the desired reaction upon the pentosan content of the wood. When the wood is then 5 cooked in suitable alkaline liquors to complete fiber liberation, the resulting pulp is substantially free from pentosans and has an exceedingly low solution viscosity. When using concentrated acid solutions, for 10 instance of from 15% to 35% acid content, the treatment may be carried out under atmospheric pressure conditions at temperatures of, say, from 20° to 40° C., but the use of dilute acid solutions of, say, an acid content of about 1% makes necessary the use of 15 much higher temperatures, which may be attained by cooking the wood while confined in a digester under super-atmospheric pressure conditions. In any event, however, the 20 initial treatment is preferably carried out under such conditions as not to effect fiber liberation, and when a sulphurous acid solution is employed, it should be substantially free from acid sulphites which react upon 25 the ligneous substance of the wood and tend to effect fiber liberation. It is possible to use an acid liquor containing, say, 1% free SO<sub>2</sub> and 2% to 4% sodium sulphate in the first step. When such a liquor is used, it is 30 best to go to a temperature of 300° to 325° F. If desired, however, acid salts such as sodium bisulphate may be added to a solution of sulphurous or sulphuric acid, as the acid constituent of such salt increases the acidity 35 of the solution, while the salt constituent retards ionization of the sulphuric acid, which may be desirable, particularly when the treatment is carried out at elevated temperature. When comparatively involatile acids 40 such as sulphuric are employed, the treatment may be advantageously carried out in open tanks under atmospheric pressure, but the use of sulphurous acid solutions at elevated temperature requires that closed digesters be used for the treatment, in order 45 to prevent the escape of sulphur dioxide from the solution.

The acid liquor associated with the wood after the treatment is a dark brown color, 50 as a result of the solution of organic matter and the hydrolysis of pentosans present in the wood to soluble sugars. At this stage, the wood is lower in pentosans than is the raw wood, and the acid liquor contains appreciable amounts of reducing sugars which 55 may have been formed by decomposition of pentosans. When a strong sulphuric or other acid solution is initially employed, it may be drained or otherwise separated from the 60 wood and employed wholly or in part for the treatment of other raw wood, but if too dilute or contaminated for reuse, its sulphur content, in the case of sulphurous or sulphuric acid solutions, may be recovered by mixing 65 it with the spent alkaline liquor recovered

from the second cooking step before the latter is subjected to the well-known recovery treatments practised in the kraft process. The acid-treated wood is of much darker color than the raw wood, usually being of 70 a reddish hue. While the wood may be readily crushed at this stage into fragments, nevertheless it is so high in ligneous matter that it does not lend itself to ready disintegration into a pulp suitable for papermaking purposes or for conversion into derivatives. The wood is preferably washed free of residual spent acid liquor before it is subjected to cooking in an alkaline liquor which 75 preferably consists of a solution of sodium hydroxide and sodium sulphide similar to that used in the kraft process. While it is possible to use a solution containing only sodium hydroxide, nevertheless it is preferable to use one containing additionally sodium sulphide, as the resulting pulp has better physical characteristics and is more easily bleachable. It is necessary, however, to use a liquor of greater alkalinity than that 80 employed in the usual refining processes, 85 wherein a raw pulp is subjected to the action of an alkaline liquor, as the acid-treated wood contains a high proportion of ligneous matter, in addition to other non-alpha cellulose components, which must be reacted 90 upon and removed by the alkali to effect fiber liberation and to produce a product of the desired high alpha cellulose content and freedom 95 from pentosans.

While a great variety of procedures falling 100 within the purview of the present invention are possible, only a typical example and certain modifications thereof will be described, as the present application is intended to cover the resulting product rather than the processes 105 which are described and claimed in other patent applications.

Spruce or other wood chips and an acid cooking liquor containing 5% free SO<sub>2</sub> are charged in the usual acid digester, and the 110 digester closed. The contents of the digester are heated to a temperature of from 225° F. to 275° F. in about three hours and are maintained at this temperature for two or three 115 hours while the pressure above the solution is regulated by the usual relief valve so as to avoid a pressure of above 75 pounds. At the end of the cooking operation, the sulphur dioxide may be released from the digester and recovered, or the digester contents may be 120 blown into the usual blowpit and the liberated sulphur dioxide may be recovered in a suitable system. The acid-cooked wood is still in chipped form, and while somewhat 125 softer than the original wood, cannot readily be reduced to a pulp. It is preferable to wash the wood free of residual spent acid liquor so as to avoid consumption of alkali. The acid-cooked chips are then cooked in a liquor containing about 1.5 pounds of alkali per cubic 130

foot, both in the form of caustic soda and sodium sulphide, the alkali poundage being calculated as active  $\text{Na}_2\text{O}$ . While all the alkali may be present in the form of caustic soda, nevertheless, as previously stated, it is preferable to have sodium sulphide present, because of the easier bleachability of the resulting pulp. The sulphidity of the alkaline liquor may amount to about 40%, which corresponds to the sulphidity of a typical kraft liquor. The alkaline cooking operation may be carried out in the usual alkaline digester and the digester contents may be heated to a maximum temperature of from 300° to 335° F. in two hours, after which the digester contents may be maintained at this temperature with the corresponding steam pressure of about 100 pounds for about two hours. At the end of the cooking operation, the wood has been converted into a pulp, so that the digester may be blown as usual, and the pulp washed free of spent liquor. The pulp at this stage has an alpha cellulose content of about 96% to 98%, a pentosan content of from 0.3 to 1, and a viscosity of 0.5 to 10. When the alkaline liquor employed to effect fiber liberation corresponds in sulphidity to the typical kraft liquor, the pulp is bleachable and may be converted to a product of high whiteness by using a bleach liquor containing only about 5% hypochlorite bleach, based on the weight of pulp. In order to preserve the high alpha cellulose content of the pulp during the bleaching operation, it is preferably to effect bleaching in a hypochlorite bleach liquor containing free alkali such as caustic soda and to maintain such liquor at a temperature of between 70° to 120° F. In lieu of hypochlorite bleach, other bleaching agents, such as permanganates, peroxides, perborates, or the like, may be employed.

A typical unbleached product produced as hereinbefore described has the following physical characteristics and composition as compared with the usual commercial unbleached sulphite and kraft pulps:

and by means of which such fiber is identified as having a solution viscosity of 10, is 1000 times as viscous as water at 20° C. Glycerin, which is often referred to as a standard when dealing with viscosity, has a viscosity value of between 8 and 10 units.

A typical bleached product produced as hereinbefore described has the following physical characteristics and composition as compared with the usual bleached sulphite and typical refined wood pulps:

|                          | Bleached product of present invention | Bleached sulphite pulp | Refined and bleached wood pulp | 75 |
|--------------------------|---------------------------------------|------------------------|--------------------------------|----|
| Strength.....            | 90 to 130                             | 125                    | 90 to 100                      |    |
| Tear resistance.....     | 250 to 400                            | 150                    | 230 to 280                     | 80 |
| Alpha cellulose (%)..... | 94 to 98                              | 84 to 86               | 92 to 94                       |    |
| Pentosans (%).....       | 0.2 to 1.0                            | 3 to 5                 | 2 to 3                         |    |
| Solution viscosity.....  | 0.2 to 1.0                            | 3 to 7                 | 3 to 10                        |    |

It is thus seen that pulps produced as herein described differ greatly from both sulphite pulp and kraft pulp in significant physical characteristics and in composition. Kraft pulp has lower tear resistance and is of lower alpha cellulose and much higher pentosan content. Sulphite pulp is much inferior in its physical characteristics, especially in its tear resistance, and has a distinctly lower alpha cellulose and higher pentosan content. Both sulphite and kraft pulp have a very much higher solution viscosity. Pulp produced as herein described is eminently suitable for use in the manufacture of high grade papers and in the preparation of various cellulose derivatives, particularly the acetates, where its substantial freedom from pentosans makes possible the production of cellulose acetate solutions of clarity and sparkle.

In some cases, it may be preferable to treat the pulp chemically, before bleaching, in order to ensure a product of high whiteness and at the same time to preserve or to increase the high alpha cellulose content realized in previous processing. For instance, the unbleached pulp may be treated for four hours and at room temperature as a 4% stock suspension in chlorine water containing from 1% to 4% chlorine, based on the weight of dry fiber, whereupon the pulp may be washed free of chlorine and reaction products and treated for about six hours and at 100° C. as a 10% stock suspension in a weakly alkaline liquor containing, say 3% to 10% caustic soda, based on the weight of dry pulp. If desired, alkalies other than caustic soda, such as sodium sulphide, may be used, and the treatment may be carried out at higher temperature and under super-atmospheric pressure. It is also possible to use temperatures materially below 100° C., if the alkalinity of the liquor is made sufficiently high,—a 5% caustic soda solution at, say, 30° C. being substantially equivalent to the use of a considerably weaker solution at much higher temperature. After the treatment with an alkaline liquor, the stock may be washed free

| 50                       | Unbleached product of present invention | Unbleached kraft pulp | Unbleached sulphite pulp |
|--------------------------|-----------------------------------------|-----------------------|--------------------------|
| Strength.....            | 90 to 130                               | 150                   | 120                      |
| Tear resistance.....     | 250 to 400                              | 250                   | 160                      |
| Alpha cellulose (%)..... | 94 to 98                                | 88 to 89              | 84 to 86                 |
| Pentosans (%).....       | 0.2 to 1.0                              | 8 to 11               | 3 to 5                   |
| Solution viscosity*..... | 0.5 to 10                               | 40 to 200             | 40 to 200                |

\* The term "solution viscosity," as herein applied to cellulose fiber, is an arbitrary one, being indicative of the viscosity of a cellulose derivative solution producible therefrom. The solution usually employed as a standard is a cuprammonium cellulose solution of definite cellulose concentration, the viscosity being determined by measuring the time of efflux of a definite volume of such solution under standard conditions through an orifice of standard size. The solution viscosity of fiber is herein given in absolute c. g. s. units, and is determined by measuring the viscosity of a solution of 6 grams of dry fiber in a cuprammonium solution composed of 225 cc. of 28% ammonia water containing 9 grams of cuprous oxide. The c. g. s. unit is employed because it is definite, denoting a viscosity 100 times that of water at 20° C., wherefore a cuprammonium cellulose solution prepared from a certain type of fiber

125

of such liquor and bleached to high whiteness with a very small amount of bleaching agent, for instance, a hypochlorite liquor containing only about 1% to 2% hypochlorite, based on the weight of the dry pulp. Preferably, a small amount of free alkali such as caustic soda is added to the bleach liquor to preserve maximum alpha cellulose content in the pulp.

In lieu of using a sulphurous acid solution in the initial treatment of the wood chips, an acid liquor containing 5% free  $\text{SO}_2$  and from 1% to 2% sodium sulphate may be employed, or one containing 5% free  $\text{SO}_2$  and 0.5% sulphuric acid, in both of which cases substantially the same cooking conditions previously given may be employed. Or an acid liquor containing 1% free  $\text{SO}_2$  and 4% sodium sulphate may be employed, in which case cooking may be effected at 300° to 325° F. An acid liquor containing 5% free  $\text{SO}_2$  and from 0.1% to 0.2% combined  $\text{SO}_2$  in the form of sodium sulphite may be employed, but with disadvantage, as it is necessary to cook at a relatively low temperature for an excessively long period of time, say, at 225% F. for from twenty-four to thirty-six hours, at the end of which time a mass of pulp of fairly low pentosan content, say 1.5% to 2.0%, and having good papermaking characteristics is obtained. This last treatment differs from all the others in which the initially treated clips remain in chip form. If paper making characteristics are not sought, the cooking operation may be carried out at a higher temperature for a shorter period of time, under which conditions the strongly acid liquor attacks the liberated cellulose fibers and so injures them that the resulting pulp is of low tear resistance. The raw pulp obtained by such a cooking operation is of low pentosan content but not high in alpha cellulose content, which may amount to, say, 85% to 86%. When such raw pulp is cooked in alkaline liquors, for instance the usual kraft liquor, the product is high in alpha cellulose and low in pentosan content. The cook may be carried out at above 100° C. and under super-atmospheric pressure, but the desired purification may also be effected in alkaline liquor at from 20° to 50° C., if the liquor is of suitable alkalinity, say, containing 5% to 8% caustic soda or caustic soda equivalent in the form both of caustic soda and sodium sulphide. It may be desirable to treat the raw pulp with chlorine water or hypochlorite liquor before treating with the alkaline liquor, to dissolve ligneous matter present in the raw pulp or render such matter more easily soluble by the alkaline liquor. The pulp may be bleached to whiteness, as already described, after treatment with the alkaline liquor.

The pentosan determinations herein given are based on the formation of furfural ( $\text{C}_4\text{H}_5\text{O}.\text{CHO}$  or  $\text{C}_5\text{H}_4\text{O}_2$ ) by means of an acid hydrolysis of the pulp, the distillation

and recovery of the furfural, and finally the determination of the amount of furfural formed (from a definite weight of dry pulp) by means of a condensation reaction of the same with phloroglucinol ( $\text{C}_6\text{H}_5\text{(CH}_2\text{)}_3$  or  $\text{C}_6\text{H}_5\text{O}_3$ ), forming furfural phloroglucide ( $\text{C}_{11}\text{H}_8\text{O}_4$ ), an insoluble precipitate. The precipitate is filtered off, washed, dried, and weighed. The weight is calculated to "pentosan" by multiplying the value by 0.7852. The pentosan value is then reported as a percent based on the original bone-dry pulp. The synopsis of the method which I employ is as follows. Add to a distilling flask fitted with a condenser, 2 grams of bone-dried shredded pulp and 100 cc. of 12% hydrochloric acid (sp. gr. 1.06). Distill slowly (rate of 30 cc. per 10 minutes) into a graduated cylinder. As each 10-cc. portion comes over, add 30 cc. acid. Continue the distillation until 270 cc. of the distillate has come over. Dissolve the proper amount of phloroglucinol (0.16 to 0.54 gram, depending upon the expected pentosan value of the pulp being tested) in 50 cc. hydrochloric acid. Add the furfural containing distillate to the phloroglucinol solution and dilute the mixture with hydrochloric acid up to a volume of 400 cc. Digest at 80-85° C. for two hours. Filter off the precipitate of furfural phloroglucide in a tared Gooch crucible and wash it with 150 cc. of distilled water at room temperature. Dry the crucible and contents for four hours at 100° C., and weigh. Weight of precipitate  $\times 39.26 =$  % pentosans.

Using the method outlined in testing normal samples of various pulps, the following values might be expected:

|                               |     |
|-------------------------------|-----|
| Cotton-----                   | 0.5 |
| Unbleached sulphite pulp----- | 4.0 |
| Bleached sulphite pulp-----   | 3.5 |
| Kraft-----                    | 8.0 |
| Groundwood -----              | 9.5 |

I claim:

1. A thoroughly bleached or whitened chemical wood pulp having an alpha cellulose content of above 96%, a pentosan content of less than 1%, and a tear resistance greater than that of unbleached kraft pulp derived from similar wood and subjected to the same degree of beating or hydration.

2. A thoroughly bleached or whitened chemical wood pulp having an alpha cellulose content of above 96%, a pentosan content of less than 1%, a tear resistance greater than that of unbleached kraft pulp derived from similar wood and subjected to the same degree of beating or hydration, and a solution viscosity markedly lower than that of a thoroughly bleached sulphite pulp derived from similar wood.

In testimony whereof I have affixed my signature.

GEORGE A. RICHTER. 130